# EUROPEAN PATENT SPECIFICATION

(11) **EP 0 605 930 B1**
(45) Date of publication and mention of the grant of the patent: **10.05.1995**
(21) Application number: 93203722.9
(22) Date of filing: 30.12.1993
(51) Int. Cl.: B28B 13/02, B28B 1/00

(54) **Method for the manufacture of dry-moulded tiles, with relative moulding plant and tile**
Verfahren zum Herstellen von trockenen Fliesen, mit seiner Formanlage und den hergestellten Fliesen
Procédé pour la fabrication de carreaux pressés à sec, avec son installation de moulage et les carreaux obtenus

(30) Priority: 08.01.1993 IT MO930002; 08.01.1993 IT MO930003
(43) Date of publication of application: 13.07.1994
(73) Proprietor: CERAMICA MIRAGE S.p.A., I-41026 Pavullo (Modena) (IT)
(72) Inventor: Montecchi, Sante,, I-41026 Pavullo nel Frignano (Modena), (IT); Chiodi, Maurizio,, I-41026 Pavullo nel Frignano (Modena), (IT)
(74) Representative: Gardi, Giuliano

(56) References cited:
- EP-A- 0 300 532
- EP-A- 0 492 733
- BE-A- 759 787
- DE-A- 2 316 481
- DE-A- 3 714 420
- DE-B- 1 070 983
- FR-A- 1 469 223
- NL-C- 74
- US-A- 1 586 805
- SOVIET PATENTS ABSTRACTS Week 8940, 15 November 1989 Derwent Publications Ltd., London, GB; AN 89-291610/40 & SU-A-1 447 681 (LVOV POLY) 30 December 1988

## Description

The invention concerns a method for the manufacture of dry-moulded ceramic tiles, with relative moulding plant and tile, namely, a new process of preparing and treating clay-based powders, or ceramic granules, possibly mixed with powdered glazes, and of feeding them into the pressing device, the actual plant where the process is carried out and the ceramic tile obtained thereby also being the object of the present invention, said ceramic tiles being suitable for tiling the inside and outside floors and walls of residential and industrial buildings and of public and private premises in general.

The prior art involves moulding methods in which mixtures of granules or clay-based powders, are extracted from a hopper by means of a driven reciprocating grid for transfer to the matrix of the press (see e.g. DE-A-2316481).

Using these methods it is not possible to obtain tiles featuring permanent decorative effects of streaking, veining and the like, in imitation of natural stone; effects of this type can only be obtained by resorting to silk-screen printing or to the application of transfers.

Plant for the manufacture of ceramic tiles includes devices for the transfer of mixtures of ceramic granules , or clay-based powders, kaolin, ground glazes, and the like, to the matrix of a ceramic-tile press consisting of a trolley with a grid for the collection and transfer of said mixtures; the trolley being longitudinally mobile with a reciprocating motion along the feeder-board of the press, between a rear loading point corresponding to the outlet for the mixtures from a hopper and a front discharge point, corresponding to the matrix of the press.

However, these devices do not allow aesthetic effects such as veining, streaking and blotching, in imitation of natural stone, to be reproduced in dry-moulded tiles: such effects only being obtainable by resorting to silk-screen printing or the application of transfers.

Moreover, silk-screen printing is a costly and cumbersome process, particularly in the case of polychrome decoration, when a separate printing device is required for each colour. Also, the decoration obtained by silk screen printing or by application of transfers permeates only a thin surface-layer of the tile; if it is worn off by scuffing or damaged by a blow, the unsightly, undecorated body of the tile is revealed. Finally, silk-screen printing and decoration with transfers only allow for the reproduction of a repetitive motif.

From the foregoing, it emerges that a solution needs to be found to the technical problem of devising a method and a relative plant for the preparation of powders, and/or clays, and/or granules, be they monochrome or polychrome, that will make it possible to obtain effects of streaking veining, or blotching, on ceramic tiles: these effects not being strictly repetitive yet conforming to a certain decorative motif or theme so that tiles of a given series are compatible with one another; finally, the process should be cost- and space-effective.

The present invention resolves the above-mentioned technical problem by adopting a method for the manufacture of ceramic tiles that involves the following steps:
1) gravity-feed of at least two types of powder down adjacent, horizontally-stratified streams having a substantially-vertical axis with a straight, preferably rectangular, cross-section, said streams flowing into a hopper to form a compact, oblong mass presenting in plan-view a plurality of more or less broad bands of similar or contrasting colour, composition and texture: said mass assuming the shape of a prism, truncated cone or pyramid, the axis of which may be inclined to the vertical plane, with a base at least equal to the surface of the faces of the tiles to be moulded; the powders forming said mass mingling progressively as the mass subsides, the degree of mingling being controlled, as required, by the depth of the mass itself, namely, the greater the depth, the greater the degree of mingling;
2) extraction by gravity from the bottom of said mass of a layer of powders at least equal in volume to that of the unmoulded tile, followed by the transfer of said layer to the moulding press: extraction having to take place by means of separate, selected feed-apertures distributed in accordance with a design motif that substantially corresponds to the distribution of the veining in the moulded tile;
3) smoothing of the face of the fired tile, before or after laying.

The expression, "types of powder", is meant to indicate powders of different colours and/or different grain-size, singly or in combination.

The feed-apertures referred to at point 2) being defined by borders in any combination of straight and/or curved or mixed lines, which may also form regular geometrical shapes: it being envisaged, furthermore, that the said feed-apertures can be selectively blocked off so as to reduce their output to a greater or lesser extent, thus facilitating the spread of the powders in the die matrix.

In a first embodiment of this method, at least three types of powder are envisaged so as to have streams flowing down a substantially vertical plane divided into layers of powder of different types forming the aforesaid prism-like mass.

The formation of said layers being achieved by means of the continuous or alternate depositing of the powders from a plurality of cylindrical columns: the straight cross-section of said columns being of symmetrical configuration with axis of symmetry advantageously horizontal, as follows:
- at least one central column for feeding the powders that figure predominantly in the composition of the tile to be moulded and which are destined to form the tile matrix;
- at least a first and second pair of alternate opposed columns for feeding the powders destined to form veins, streaks, or blotches;
it being envisaged that the distribution of powders that go to form the prism-like mass occurs by means of reciprocating or synchronous traverse of said columns in a direction orthogonal or parallel to that of extraction of the bottom layer of powders; the powders in each column forming the layers of each said stream; the angle formed between the direction of motion of translation of the columns and the axis of symmetry of their plan configuration being between 0° and 180°.

The motion of translation of said columns possibly being complemented by rotation about the longitudinal axis, the degree of rotation being pre-established for each run and varying between fractions of a rotation and one or more full rotations.

In a second embodiment of the method, the feeding of the powders from at least one column being intermittent, in order to obtain, for example, sporadic, randomly-distributed blotches of colour in the tile being moulded.

The invention also includes a plant for the dry-moulding of ceramic tiles, consisting of a die fed by a slide, or trolley, that is cranked to and fro along the feeder-board of the die-matrix in order to transport to the matrix itself a predetermined quantity of powders extracted by gravity from the lower outlet of a hopper by means of a grid fixed to said slide; it being envisaged that a multiple powder distributor, having at least two feed-ducts and driven to travel with a horizontal, reciprocating motion, be mounted above the upper loading aperture of said hopper; said grid consisting of a plurality of vertical baffles forming separate, selected feed apertures for the powders and conforming to a motif prefiguring that formed by the distribution of veining in the tile; said baffles presenting in plan view straight lines or broken curves, or any combination of the two, and being oriented with respect to the direction of travel of the slide at an angle of between 0° and 90°: said angle being constant or variable between the baffles and between consecutive sections of each baffle, in order to form outlets for the powders to pass through, arranged according to a motif featuring stripes, and/or polygons with curved sides, and/or geometrical shapes.

The tile obtained by this method consisting of a ceramic body obtained by dry-moulding in which the decorative effects of veining, and/or streaking, and blotching, intermingle and penetrate the possibly homogeneous body of the tile to a substantial depth of at least 2mm and even to its very base.

The advantages offered by the invention are: the realisation of original, choice and durable aesthetic effects on the tiles,consisting of streaking and veining, and blotching, colour-coordinated with the tile body or in contrast with it; avoidance of repetitiveness in the chromatic effect while preserving the same pattern of veining in the tiles of a given series; moderate cost; modest overall dimensions.

Some ways of carrying out the invention are illustrated, by way of example, in the eleven tables of drawings attached, in which: Figure 1 is a partly-sectional side view of the plant for feeding the powders to the moulding press; Figure 2 is a partly-sectional left view of Fig. 1, showing the device for traversing the multiple distributor; Figure 3 is a plan view of the feeder board of the die, in the version for the moulding of one tile per cycle, for example in the format 40 cm x 40 cm; Figure 4 is the enlarged straight cross-section IV - IV of Figure 1 showing the configuration of the conduits in the five-channel embodyment of the multiple distributor, for example for three colours; Figure 5 is a schematic diagram of the distribution of powders in the hopper after a single traverse of the multiple distributor; Figure 6 is a schematic vertical section of the hopper provided with a first embodiment of the distributor having motion orthogonal to the direction of travel of the slide, the hopper showing the stratifying of the powders after to-and-fro traverse of the distributor in Fig. 4; Figure 7 is a cross-section like that of Figure 4 but in the eight-channel embodyment, for example for five colours; Figure 8 is a plan view, from below, of a first embodiment of the grid for extracting the powders from the hopper and transporting the same to the moulding press, with wavy baffles inclined obliquely to the direction of travel of the trolley; Figure 9 is a plan view, from below, of a second embodiment of the grid, with oblique wavy baffles interspersed with blocking elements; Figure 10 is a plan view, from below, of a third embodiment of the grid with the baffles arranged in a pattern of variously-shaped polygons and interspersed with blocking elements; Figures 11, 12, 13 are plan views from below of a fourth, fifth and sixth embodiment of the grid with their geometrical patterns defined, respectively, by parallel baffles, at right- angles to the direction of travel of the trolley, by straight baffles in a criss-cross configuration and by baffles that are circular in cross-section; Figure 14 is a schematic vertical section of the hopper provided with a second embodiment of the distributor having motion parallel to the direction of travel of the slide; Figure 15 is a plan view of the hopper of Figure 14; Figure 16 is a schematic plan view of a ceramic tile according to the invention; Figure 17 is section XVII-XVII of Figure 16, in which the various shadings correspond to various colours or powders.

The figures show: the plant 1 for the preparation of the powders and their transfer to the moulding press 2; the feeder-board 3 of the die of the press 4 along which a slide 5 travels with a reciprocating motion, having a pair of sides 6 designed to slide between longitudinal guides 7 with the interposition of two pairs of opposed rolling elements 8; a device 9 featuring a crank and slotted link for driving the slide 5; a grid 10 for receiving the powders from the lower aperture of a hopper 11 and transporting them in a controlled manner to a die-matrix 12: said matrix advantageously having a base-plate capable of vertical movement between its top position, when it lines up with the feeder-board 3 of the press, and its bottom position, when the matrix is charged before a die-punch 13 descends; a removable frame 14,(Figure 3) of the grid 10, slotted into the front section of the slide 5; a cleaning device 15 for the feeder-board operating after each pressing, comprising a cylindrical rotating brush, pivotally-mounted at the front end of the pair of sides 6: said brush being capable of being raised clear of the feeder surface on the return run by means of a device featuring a pair of articulated parallelograms, not shown, operated by a pneumatic cylinder 16 having its shaft hinged to a crosspiece 17 linking the connecting rods of the said parallelograms; the motor 18 rotating said cleaning element 15 by means of two pairs of pulleys 19 connected by a pair of drive belts 20; a slot 21 in a rear cross-member 22 linking the sides 6 of said slide, said slot acting as a guide for a cursor 23 mounted on a roller at the end of the crank 24; a bar 25 for expelling the moulded tiles fixed to the leading edge of the slide 5; a scraper-blade 26 oscillating in a vertical slot of a front cross-member 27 of the slide 5.

Inserted in the upper section of the hopper 11 is a dispenser 28 of a multiple distributor 29 for the powders, said distributor being gravity-fed by means of a plurality of pairs of conduits 30, 31, 32, the upper sections of which are flexible and lead from the containers 33, 34, 35, respectively, of the powders A, B, C: it being envisaged that the quantity of powder in said containers 33, 34, 35, respectively, be kept constant by means of a level-compensating device, comprising, for example, interception valves triggered by level-sensors, not shown, mounted on the feed-ducts of the containers themselves: the pair of central conduits 30 being advantageously connected to a single central conduit 30a in the lower section of the sleeve 36 of the multiple distributor 29.

The pairs of conduits 30, 31, 32, converging in the sleeve 36 of the multiple distributor 29, are located centrally, in the case of the pair of conduits 30 destined to carry the powder for the matrix of the tile, and in diametrically-opposite positions, in the case of the pairs of conduits carrying the powder for veining: it being possible for said powders to be of very different, or for example homogeneous, grain-size, or to consist of mixtures of granules and powder, of the same or different colour, or in polychromatic combinations.

The dispenser 28, formed by the extension downwards of the sleeve 36 enveloping the bottom sections of the pairs of conduits 30, 31, 32, has its mouth 28a parallel to the feeder board 3 of the moulding press to ensure that the hopper 11 is uniformly charged.

The pairs of conduits 30, 31, 32 together defining a plurality of columns destined to form the layers of each stream as described in step 1) of the method according to the invention.

In particular, powders A, B, C flow down a plurality of adjacent streams 33b corresponding to said columns, said streams being separated by ideal sustantially vertical planes 33a: each stream, having a straight rectangular cross-section equal in length to the hopper 11, consisting of superimposed sections of a plurality of layers 33c of powders A, B, C.

Layers 33c being defined by ideal planes 50 inclined down in the direction Y of extraction of the slide 5 at an angle that increases as the distance of the generic layer 50 from the lower layer decreases and as the rate of extraction by the slide drops.

The figures also show: the depth S of the powders in the hopper 11, advantageously ranging between about 10cm and about 25cm and adjustable by varying the axial position of the dispenser 28 by means of an actuator, not shown: increased depth corresponding to greater degree of mingling between the streams 33b relative to each column; a bracket 37 clamping the ring-shaped projection of the sleeve 36 to a trolley 38 sliding bilaterally, by means of two pairs of opposed wheels 39, on a pair of transverse guiderails 40 fixed to the framework; an enclosed block-chain 41 on a pair of crownwheels 42, one of which driven, having the upper section fixed to said trolley so as to move it: the length of travel L of the trolley being equal to the transverse dimension L1 of the hopper 11 less the transverse dimension L2 of the dispenser 28 of the distributor 29; a plurality of columns D, E, F, G, H of powders, or granules, of different types, singly or in combination, monochrome or polychrome, inserted in respective couples 51, 52, 53 of conduits analogous to those relative to the powders B, C,in the case of the columns of powders D, E, F: the central conduits 54, 55 being fed with columns of powders G, H, of different types, for example in order to obtain a streaky effect with a greater number of colours; a base frame 43 of the hopper 11 featuring a peripheral lip 44 to act as a dry seal against the upper surface of the slide 5 and so prevent powder spillage, when said slide is at the front-stop charging the die matrix 12; a plurality of baffles 45,(Figure 8), dividing the grid 10 into zones for the containment of the powders and for their controlled release into the die matrix: said baffles having contours in plan view of any combination of wavy curves, either continuous or interrupted, the ends being fixed to the frame 14. The plan configuration of the baffles 45 prefigures the distribution of the veining in the tile in that it defines the separate feed apertures selected, as described in step 2) of the method according to the invention; the axis Z1 of one of the said baffles forming an angle B1 to the direction Z2 of travel of the grid 10, the term axis being used to indicate the straight line representing the mean inclination of the contour of a baffle or also of only a section of it: the angle B1 being variable between 0° and 180° and capable of remaining constant for the baffles of a given grid or of varying, in a random or repetitive manner, over single or successive sections of any one baffle, so as to create random or geometrical shapes, for instance touching circles 46, (Figure 13), consecutive squares or parallelograms 47, (Figure 12), parallel lines 48 (Figure 11), or whatever is appropriate; blocking elements 49 interposed between adjacent baffles forming zones where the downward flow of powders during the charging of the grid is blocked and such as to cause the powders to spread out when the base of the matrix is lowered: the thickness of said baffles, varying, from baffle to baffle or from section to section of one and the same baffle, as required, between a few millimetres to several centimetres, for example even ten or more, in the latter case functioning as a substitute for or a complement to the blocking elements 49.

The axis of symmetry Z3, (Figure 4) of the straight cross-section of the multiple distributor 29 forms an angle B2 with the direction of travel of the trolley 38: the size of the angle B2 ranging between 0° and 180°.

The depth of the baffles 45, determining the load capacity of the grid, is such as to allow a quantity of powder to be collected that is anyway greater than the volume of the layer of powder to be moulded that can be contained in the die-matrix 12 and may even amount to twice that volume, for example.

The distribution of the baffles 45 determines the nature of the veining of the tile, for example a diagonal configuration seen in Figures 8, 9 determines a correspondingly-diagonal pattern of veining, while the distribution of the baffles in asymmetrical polygons with varying contours as seen in Figure 10 produces a blotched effect.

Veining can be extended to the whole thickness of the tile if the die matrix is charged in a single layer, or be limited to just a part of the thickness of the tile, as when charging with several layers, the minimum thickness being about 2mm.

### Examples.

Realisation of a tile using a grid as in the first embodiment (Figure 8).

| Composition (by volume): | |
|---|---|
| powder A (red) | 46% |
| powder B (black) | 27% |
| powder C (yellow) | 27% |
| grain-size | from 0.01 to 1.8mm |
| mean humidity | from 5 to 6.5% |
| format | 40cm x 40cm |

| The parameters of the forming process being the following: | |
|---|---|
| equivalent diameter of central column 30a | 71mm |
| diameter of each column 31 | 38mm |
| diameter of each column 32 | 38mm |
| depths of powders in hopper 11 | from 15 to 20cm |
| size of angle B2 | 15° |

| Extraction parameters: | |
|---|---|
| travel of slide 5 | 720mm |
| mean rate of extraction of slide 5 | 102m/min |
| period | 1.18s |

The charging of the die matrix 12 is accomplished by the lowering of the base-plate of the matrix when the slide is at the front-stop.

The moulding process is as follows: when, by rotation of the crank 24, the slide 5 is recalled from the front-stop position, where charging of the die-matrix 12 takes place, and the back edge of the frame 14 slides under the front edge of the hopper 11, the powder contained in the hopper itself falls by gravity into the separate selected feed outlets 45a formed by the baffles 45 and onto any residue of surplus powder remaining after the charging of said die-matrix: the rate of travel of the slide being coordinated with the rate of fall of the powders so as to effect the gradual replenishing of the grid 10 on its return run; a subsequent rotation of the crank then advances the slide towards the die-matrix and the charging process is repeated.

The moulded tiles are then conveyed to the kiln for firing and subsequent grinding, which may take place after laying.

The powders are gradually consumed along ideal planes 50, (Figure 6) inclined forwards and down towards the feeder-board 3 of the press; the reserve of powders being replenished at every cycle by a traverse of the multiple distributor 29, clamped to the trolley 38, over the whole length of the hopper 11; the quantity of powders deposited on each run of the trolley being such as to restore the depth S of powders in the hopper 11. The powders are thus distributed in the hopper 11 in streams 33b built up in layers 33c: the central stream consisting substantially of any powder being introduced in greater proportion, the lateral streams consisting of alternate layers 33c of powders in lesser proportions: the degree of mingling between layers and/or adjacent streams depending on the ratio between the volume of powder consumed at each cycle and the depth S.

It being noted that, with the same grid, if the rate of travel of the slide 5 is increased as it passes under the hopper 11, veining is thinner and longer and the colour contrast lessens: if the rate of travel is decreased, blotchy veining is achieved. Furthermore, if powders of different grain-size are used, the larger particles tend to flow, with the result that greater colour contrasts can be obtained.

It being possible to feed the powder through the conduits, or columns, 30, 31, 32, 51, 52, 53, 54, 55 intermittently, thus allowing the number of colours and/or grain-sizes in the powder in a given series of tiles being formed to be varied in a controlled fashion.

In another embodiment of the invention, the multiple distributor 29 may, in addition to running back and forth to restore the depth S of powders in the hopper, be enabled to rotate, continuously or intermittently, around its own longitudinal axis: this makes it possible to achieve aesthetic effects which are further enhanced by the greater degree of mixing between the powders.

In this case, the dispenser 28 clamped to the trolley 38 must be pivotally coupled to the sleeve 36 on a plane X orthogonal to the axis of the sleeve itself, so as to allow the rotation of the sleeve through a predetermined angle, equal to one rotation or to a fraction of a rotation: it being possible to achieve the rotary action of the distributor by means of a pneumatic cylinder, reduction unit, cam device, or other appropriate means.

In a further embodiment of the invention shown in Figures 14, 15, a second embodiment of the multiple distributor 129 comprises a casing 129a extending substantially the whole width of the hopper 11, said casing enclosing a plurality of substantially vertical conduits 130, 131, 132 alligned along its length.

The distributor 129, coupled with driving means 153 has a bottom exit which co-operates with a flow control member comprising a shelf 151, adjacent to the top of the hopper 11, which closes the bottom exit of said distributor when not in operation (operative position in dotted line).

The conduits have extendable outlets 130a, 131a, whose position with respect to the bottom exit of said distributor 129 determines the quantity of powders introduced in the casing 129a: by adjusting the position of the extendable outlets it is possible to slightly change the pattern of the tile in a very easy way.

The hopper 11 may be provided with a plurality of parallel vanes 152, said vanes are pivotable in order to deflect the flow of powder in substantially separated streams.

In practice, the dimensions and details of execution may be different from but technically equivalent to those described without departing from the scope of the present invention.

## Claims

1. Method for the manufacture of dry-moulded ceramic tiles, comprising the preparation of the powders, flowing the powders into a hopper, transfer of the powders to a pressing device, pressing the powders and kiln-firing, characterised in that
- at least two types of powder or granules are charged to the hopper and form a mass of material in granules or powder comprising adjacent streams (33b) which, at least in the upper part of said mass, are distinct from one another;
- a layer of granules or powder is extracted by gravity from the bottom of said mass of material by means of a grid (10) defining separate, selected feed apertures (45a), these feed apertures (45a) being distributed in accordance with a design motif of the moulded tile.

2. Method as claimed in claim 1, characterized in that said streams (33b) flow down a substantially-vertical axis.

3. Method as claimed in claim 1 or 2, characterized in that said streams (33b) are formed by superimposed layers of the at least two types of said powders.

4. Method as claimed in claim 1, 2 or 3, characterized in that said mass is in the shape of a prism or truncated pyramid, the axis of which may be inclined to the vertical plane, said streams mingling in said mass.

5. Method as claimed in claim 4, characterized in that the depth (S) of said mass is determined by the degree of merging envisaged between said streams (33b).

6. Method as claimed in claim 1 or 4, characterised by the fact that said streams (33b) have a substantially rectangular cross-section.

7. Method as claimed in claims 1 or 4, characterized in that said feed apertures (45a) are distributed according to a motif substantially corresponding to the distribution of veining, streaking and blotching in the moulded tile.

8. Method as claimed in claim 1 or 4, characterized in that said powders differ from each other in colour. possibly, in grain size.

9. Method as claimed in claim 1 or 4, characterized in that said powders differ from each other in grain size.

10. Method as claimed in one or more of the foregoing claims, characterized in that said lower layer of powders is at least equal in volume to that of the unmoulded tile.

11. Method as claimed in one or more of the foregoing claims, characterized in that said feed apertures (45a) are defined by any combination of straight contours.

12. Method as claimed in one or more of claims 1 to 10, characterized in that said feed apertures (45a) are defined by any combination of curved contours connected, or not, by straight sections.

13. Method as claimed in one or more of the foregoing claims, characterized in that said feed apertures (45a) are blocked off so as to reduce their output to a greater or lesser extent, thus facilitating the spread of the powder in the pressing device.

14. Method as claimed in claim 3, characterized in that said streams (33b) stratified in layers (6) are formed by the alternate deposition of powders from columns having substantially-vertical axes.

15. Method as claimed in claim 14, characterized in that said alternate deposition of the powders is achieved by alternating and, possibly, synchronous traverse of said columns in a direction orthogonal to the direction (Y) of extraction of the lower layer of powders.

16. Method as claimed in claim 14, characterized in that said alternate deposition of the powders is achieved by alternating and, possibly, synchronous traverse of said columns in a direction parallel to the direction (Y) of extraction of the lower layer of powders.

17. Method as claimed in claim 15, or 16, characterized in that said alternating traverse is complemented by a rotation of the columns about an axis parallel to the axes of the columns themselves; the degree of said rotation being predetermined up to a maximum value of at least one full turn.

18. Method according to one or more of the preceeding claims, characterized in that at least one of said columns is fed intermittently.

19. Plant for the moulding of ceramic tiles for carrying out the method as claimed in claims 1 to 18, including a die (12, 13) fed by means of a slide (5) or trolley, cranked to and fro along the feeder-board (3) or the die-matrix (12) in order to transport to the matrix itself a predetermined quantity of powders extracted by gravity from the lower outlet of a hopper (11) by means of a grid fixed to said slide, characterized in that a multiple powder distributor (29; 129), having at least two ducts for feeding the columns of powders or granules to the hopper, is mounted above the upper loading aperture of said hopper (11) and is driven to travel with a horizontal reciprocating motion, and in that the grid (10) is formed of a plurality of vertical baffles (45, 46, 47, 48) defining separated, selected feed apertures (45a) for the powders and conforming to a motif prefiguring that formed by the distribution of veining, streaking and blotching in the tile.

20. Plant as claimed in claim 19, characterized in that said multiple distributor consists of a sleeve (36) in which at least two conduits defining said at least two ducts for feeding the columns of powders to the hopper (11) converge.

21. Plant as claimed in claim 20, characterized in that the straight cross-section of said multiple distributor (29) is symmetrical with respect to a horizontal axis (Z3) forming an angle (B2) with the direction of travel of the distributor: said angle being variable between 0° and 180°.

22. Plant as claimed in claim 20 or 21 characterized in that said multiple distributor (29) has five conduits inside said sleeve (36) comprising a central conduit (30a) and two opposed alternate pairs of peripheral conduits (31).

23. Plant as claimed in claim 20 or 21, characterized in that said multiple distributor (29) has eight conduits inside said sleeve comprising three opposed alternate pairs of peripheral conduits (51, 52, 53) and two central conduits (54, 55).

24. Plant, as claimed in claim 19, characterized in that the multiple distributor (129) comprises a casing (129a) extending substantially the whole width of the hopper (11), said casing enclosing a plurality of conduits (130, 131, 132) along its length.

25. Plant, as claimed in claim 24, characterized in that, the distributor (129) has a bottom exit which co-operates with a flow control member.

26. Plant, as claimed in claim 25, characterized in that, the flow control member comprises a shelf (151), adjacent to the top of the hopper (11), which closes the bottom exit of said distributor.

27. Plant, as claimed in claim 24, characterized in that the conduits have extendable outlets (130a, 131a).

28. Plant as claimed in any of claims 24 to 27, characterized in that said hopper (11) is provided with a plurality of parallel vanes (152).

29. Plant, according to claim 28, characterized in that, the vains are pivotable.

30. Plant according to any of claims 19 to 29, characterized in that the distributor (29; 129) is driven to travel with a horizontal reciprocating motion.

31. Plant, according to claim 30, characterized in that the direction in which the distributor is driven is parallel to the direction (Y) of travel of the grid.

32. Plant, according to claim 30, characterized in that, the direction in which the distributor is driven is orthogonal to the direction (Y) of travel of the grid.

33. Plant as claimed in one or more of claims 19 to 32, characterized in that said grid (10) has baffles (45) presenting in plan view any combination of wavy curved lines; the axis (Z1) of each baffle forming an angle (B1) with respect to the direction (Z2, Y) of travel of the grid between 0° and 180°: said angle not necessarily being constant between the baffles.

34. Plant as claimed in claim 33, characterized in that said angle may vary from section to section of one and the same baffle.

35. Plant as claimed in claim 33, characterized in that said grid (10) has baffles (47, 48) presenting in plan view any combination of straight lines.

36. Plant as claimed in claim 33, characterized in that said grid (10) has baffles presenting in plan view curved lines such as to define a pattern of touching circumferences.

37. Plant as claimed in any one of claims 33 to 36, characterized in that said grid (10) has blocking elements (49) interposed between adjacent baffles to block the downflow of powders from the hopper (11).

38. Plant as claimed in any of claims 33 to 37, characterized in that the depth of the baffles of said grid is such as to allow a volume of powders to be extracted from the lower section of the hopper (11) that is greater than the volume of the tile to be moulded.

39. Plant, according to claim 38, characterized in that, the volume of the powders to be extracted is twice the volume of the tile to be moulded.

40. Plant as claimed in claim 24, characterized in that the sleeve (36) of said multiple distributor (29) extends downwards to form a dispenser (28) with a mouth (28a) parallel to the feeder-board (3) of the die.

41. Plant as claimed in claim 40, characterized in that the distance between said mouth and said feeder-board, determining the depth (S) of the powders in the hopper (11) is between about 10 cm and about 25 cm.

42. Plant as claimed in claim 33, characterized in that the sleeve (36) of said multiple distributor (29) has a ring-shaped projection for coupling to a bracket (37) mounted on a trolley (38) sliding bilaterally on a pair of transverse guiderails (40).

43. Plant as claimed in claim 32, characterized in that said conduits (30, 31, 32) are flexible in their upper sections to enable them to be inserted into relative powder containers (34, 35, 36) fed by means of a level-compensator device.

44. Plant as claimed in claim 32, characterized in that a slide (5), on which is mounted the grid (10) for the extraction and transfer of the powders, is driven by means of a crank and slotted link (9) to run to and fro beneath the lower section of said hopper (11).

45. Plant as claimed in claim 40, characterized in that said sleeve (36) is pivotally mounted on the dispenser (28) along a transverse plane (X) orthogonal to the longitudinal axis of said sleeve to allow it to rotate through a predetermined angle in its traverse of the hopper (11) by means of an actuator.

46. Plant as claimed in claim 42, characterized in that said conduits (30, 31, 32, 50, 51, 52, 53, 54, 55) are fixed inside said sleeve (36); said dispenser (28) being integral with said trolley (38).

47. Plant as claimed in claim 19, characterized in that the thickness of said baffles may vary from section to section of one and the same baffle between a few millimetres to several or more centimetres.

48. Plant as claimed in claim 47, characterized in that said baffles vary in thickness from one another.

49. Plant as claimed in claim 40, characterized in that the traverse (L) of said dispenser (28) is equal to the transverse dimension (L1) of the hopper (11) less the transverse dimension (L2) of the dispenser itself.

50. Plant as claimed in claim 19, characterized in that a cylindrical rotating brush (15) is mounted on the front part of said slide (5) by means of a pair of articulated parallelograms interconnected by means of a cross-member (17) and driven by a pneumatic cylinder (16).

51. Plant as claimed in any of the preceding claims characterized in that said columns are arranged in a symmetrical configuration having a straight cross-section with at least one axis of symmetry (Z3) advantageously horizontal, said configuration comprising:
- at least one central column (30, 30a, 55) for the ducting of powders destined to form the matrix of the tile;
- at least one first (31, 51) and one second (32, 52) pair of alternate opposed columns for ducting the powders destined to form the veining or blotching of the tile.

52. Plant as claimed in claim 51, characterized in that said symmetrical configuration of the columns comprises at least one central column (30a, 54, 55) and at least one alternate opposed pair of peripheral columns (31, 32, 51, 52, 53).

53. Plant as claimed in claim 51 or 52, characterized in that the axis of symmetry (Z3) of said straight cross-section forms an angle (B2) of between 0° and 180° with the direction (Z4) of the traverse of the columns.

54. Tile, obtainable by the method as claimed in claims 1 to 18, having a surface provided with veining, streaking, and/or blotching and consisting of a dry-moulded ceramic body, characterized in that the veining, streaking and/or blotching, intermingle and penetrate the tile matrix to at least a substantial depth of the whole thickness.

55. Tile as claimed in claim 54, characterized in that said substantial depth is equal to at least 2 mm.

## Patentansprüche

1. Verfahren zum Fertigen von trocken geformten Keramikfliesen, einschließlich der Vorbereitung der Pulver, dem Eingeben des Pulvers in einen Vorratsbehälter, des Transfers der Pulver in eine Preßvorrichtung, des Pressens der Pulver und des Brennens in einem Kiln-Ofen,
dadurch gekennzeichnet, daß
- wenigstens zwei Sorten von Pulver oder Körnchen in den Vorratsbehälter geladen werden und eine Materialmasse aus Körnchen oder Pulver mit benachbarten Strömen (33b) formen, die wenigstens in dem oberen Teil der Masse voneinander verschieden sind,
- eine Schicht von Körnchen oder Pulver mittels eines getrennte, ausgewählte Zufuhröffnungen (45a) definierenden Gitters (10) von dem Boden der Materialmasse durch Schwerkraft abgegeben wird, wobei diese Zufuhröffnungen (45a) in Übereinstimmung mit einem Motiventwurf der geformten Fliese verteilt sind.

2. Verfahren nach Anspruch 1, dadurch gekennzeichnet, daß die Ströme (33b) in einer im wesentlichen vertikalen Achse nach unten fließen.

3. Verfahren nach Anspruch 1 oder 2, dadurch gekennzeichnet, daß die Ströme (33b) durch übereinanderliegende Schichten der wenigstens zwei Sorten der Pulver gebildet werden.

4. Verfahren nach Anspruch 1, 2 oder 3, dadurch gekennzeichnet, daß die Masse die Form eines Prismas oder eines Pyramidenstumpfes aufweist, dessen bzw. deren Achse zu der vertikalen Ebene geneigt sein kann, wobei sich die Ströme in der Masse vermengen.

5. Verfahren nach Anspruch 4, dadurch gekennzeichnet, daß die Tiefe (S) der Masse durch den Grad an angestrebter Vermengung zwischen den Strömen (33b) bestimmt ist.

6. Verfahren nach Anspruch 1 oder 4, gekennzeichnet durch die Tatsache, daß die Ströme (33b) einen im wesentlichen rechtwinkligen Querschnitt aufweisen.

7. Verfahren nach Anspruch 1 oder 4, dadurch gekennzeichnet, daß die Zufuhröffnungen (45a) entsprechend einem Motiv verteilt sind, das im wesentlichen der Verteilung von Aderung, Maserung und Flecken in der geformten Fliese entspricht.

8. Verfahren nach Anspruch 1 oder 4, dadurch gekennzeichnet, daß die Pulver sich voneinander in der Farbe und möglicherweise in der Korngröße unterscheiden.

9. Verfahren nach Anspruch 1 oder 4, dadurch gekennzeichnet, daß sich die Pulver voneinander in der Korngröße unterscheiden.

10. Verfahren nach einem oder mehreren der vorhergehenden Ansprüche, dadurch gekennzeichnet, daß die untere Schicht von Pulvern im Volumen wenigstens gleich dem Volumen der ungeformten Fliese ist.

11. Verfahren nach einem oder mehreren der vorhergehenden Ansprüche, dadurch gekennzeichnet, daß die Zufuhröffnungen (45a) durch eine beliebige Kombination von geraden Umrissen definiert sind.

12. Verfahren nach einem oder mehreren der Ansprüche 1 bis 10, dadurch gekennzeichnet, daß die Zufuhröffnungen (45a) durch eine beliebige Kombination von gekrümmten Umrissen definiert sind, die durch gerade Abschnitte miteinander verbunden sind oder auch nicht.

13. Verfahren nach einem oder mehreren der vorhergehenden Ansprüche, dadurch gekennzeichnet, daß die Zufuhröffnungen (45a) versperrt werden, um so ihren Ausstoß um ein größeres oder geringeres Maß zu reduzieren und die Verteilung des Pulvers in der Preßvorrichtung zu erleichtern.

14. Verfahren nach Anspruch 3, dadurch gekennzeichnet, daß die in Schichten (6) geschichteten Ströme (33b) durch die alternierende Ablagerung von Pulvern aus Säulen mit im wesentlichen vertikalen Achsen gebildet werden.

15. Verfahren nach Anspruch 14, dadurch gekennzeichnet, daß die alternierende Ablagerung der Pulver erreicht wird, indem die Säulen alternierend und möglicherweise synchron in einer Richtung orthogonal zu der Richtung (Y) der Abgabe der unteren Schicht von Pulvern traversiert werden.

16. Verfahren nach Anspruch 14, dadurch gekennzeichnet, daß die alternierende Ablagerung der Pulver erreicht wird, indem die Säulen alternierend und möglicherweise synchron in einer Richtung parallel zu der Richtung (Y) der Abgabe der unteren Schicht von Pulvern traversiert werden.

17. Verfahren nach Anspruch 15 oder 16, dadurch gekennzeichnet, daß das alternierende Traversieren durch eine Drehung der Säulen um eine Achse parallel zu den Achsen der Säulen selbst ergänzt wird, wobei der Grad der Rotation bis zu einem Maximalwert von wenigstens einer vollen Umdrehung vorbestimmt ist.

18. Verfahren nach einem oder mehreren der vorhergehenden Ansprüche, dadurch gekennzeichnet, daß wenigstens eine der Säulen intermittierend gespeist wird.

19. Anlage zum Formen von Keramikfliesen, für die Durchführung des Verfahrens nach den Ansprüchen 1 bis 18, mit einem Stempelwerkzeug (12, 13), das mittels eines Schlittens (5) oder Förderwagens gespeist wird, der längs der Zufuhrseite (3) oder der Stempel-Matrix (12) hin- und herbewegt wird, um zu der Matrix selbst eine vorbestimmte Menge von Pulvern zu transportieren, die mittels eines an dem Schlitten befestigten Gitters durch Schwerkraft aus dem unteren Auslaß eines Vorratsbehälters (11) abgegeben werden, dadurch gekennzeichnet, daß ein Mehrfach-Pulververteiler (29; 129) mit wenigstens zwei Durchführungen zum Zuführen der Säulen von Pulvern oder Körnchen zu dem Vorratsbehälter oberhalb der oberen Ladeöffnung des Vorratsbehälters (11) angeordnet und derart angetrieben ist, daß er sich mit einer horizontalen, hin- und hergehenden Bewegung bewegt, und
dadurch, daß das Gitter (10) aus einer Vielzahl von vertikalen Prallblechen (45, 46, 47, 48) gebildet ist, die getrennte, ausgewählte Zufuhröffnungen (45a) für die Pulver definieren und einem Motiv entsprechen, das das Vorbild für das durch die Verteilung von Aderung, Maserung und Flecken in der Fliese gebildete Motiv ist.

20. Anlage nach Anspruch 19, dadurch gekennzeichnet, daß der Mehrfachverteiler aus einer Hülse (36) besteht, in der wenigstens zwei die wenigstens beiden Durchführungen definierende Rohrleitungen zum Zuführen der Säulen von Pulvern zu dem Vorratsbehälter (11) konvergieren.

21. Anlage nach Anspruch 20, dadurch gekennzeichnet, daß der gerade Querschnitt des Mehrfachverteilers (29) bezogen auf eine horizontale Achse (Z3) symmetrisch ist, die mit der Richtung der Bewegung des Verteilers einen Winkel (B2) bildet, wobei der Winkel zwischen 0° und 180° veränderbar ist.

22. Anlage nach Anspruch 20 oder 21, dadurch gekennzeichnet, daß der Mehrfachverteiler (29) fünf Rohrleitungen innerhalb der Hülse (36) aufweist, zu denen eine zentrale Rohrleitung (30a) und zwei einander gegenüberliegende, sich abwechselnde Paare von äußeren Rohrleitungen (31) zählen.

23. Anlage nach Anspruch 20 oder 21, dadurch gekennzeichnet, daß der Mehrfachverteiler (29) acht Rohrleitungen innerhalb der Hülse umfaßt, zu denen drei einander gegenüberliegende, sich abwechselnde Paare von äußeren Rohrleitungen (51, 52, 53) und zwei zentrale Rohrleitungen (54, 55) gehören.

24. Anlage nach Anspruch 19, dadurch gekennzeichnet, daß der Mehrfachverteiler (129) ein Gehäuse (129a) umfaßt, das sich im wesentlichen über die gesamte Breite des Vorratsbehälters (11) erstreckt, wobei das Gehäuse eine Vielzahl von Rohrleitungen (130, 131, 132) längs seiner Länge einschließt.

25. Anlage nach Anspruch 24, dadurch gekennzeichnet, daß der Verteiler (129) einen Bodenauslaß aufweist, der mit einem Flußsteuerteil zusammenwirkt.

26. Anlage nach Anspruch 25, dadurch gekennzeichnet, daß das Flußsteuerteil ein neben der Oberseite des Vorratsbehälters (11) angeordnetes Brett (151) umfaßt, das den Bodenauslaß des Verteilers verschließt.

27. Anlage nach Anspruch 24, dadurch gekennzeichnet, daß die Rohrleitungen verlängerbare Auslässe (130a, 131a) aufweisen.

28. Anlage nach einem der Ansprüche 24 bis 27, dadurch gekennzeichnet, daß der Vorratsbehälter (11) mit einer Vielzahl von parallelen Flügeln (152) versehen ist.

29. Anlage nach Anspruch 28, dadurch gekennzeichnet, daß die Flügel schwenkbar sind.

30. Anlage nach einem der Ansprüche 19 bis 29, dadurch gekennzeichnet, daß der Verteiler (29; 129) so angetrieben ist, daß er sich mit einer horizontalen, hin- und hergehenden Bewegung bewegt.

31. Anlage nach Anspruch 30, dadurch gekennzeichnet, daß die Richtung, in der der Verteiler angetrieben ist, parallel zu der Richtung (Y) der Bewegung des Gitters ist.

32. Anlage nach Anspruch 30, dadurch gekennzeichnet, daß die Richtung, in der der Verteiler angetrieben ist, orthogonal zu der Richtung (Y) der Bewegung des Gitters ist.

33. Anlage nach einem oder mehreren der Ansprüche 19 bis 32, dadurch gekennzeichnet, daß das Gitter (10) Prallbleche (45) umfaßt, die in der Draufsicht eine beliebige Kombination von wellig gekrümmten Linien aufweisen, wobei die Achse (Z1) eines jeden Prallbleches bezogen auf die Richtung (Z2, Y) der Bewegung des Gitters einen Winkel (B1) zwischen 0° und 180° bildet und der Winkel unter den Prallblechen nicht notwendigerweise konstant ist.

34. Anlage nach Anspruch 33, dadurch gekennzeichnet, daß der Winkel von Abschnitt zu Abschnitt ein und desselben Prallbleches variieren kann.

35. Anlage nach Anspruch 33, dadurch gekennzeichnet, daß das Gitter (10) Prallbleche (47, 48) aufweist, die in der Draufsicht eine beliebige Kombination von geraden Linien zeigen.

36. Anlage nach Anspruch 33, dadurch gekennzeichnet, daß das Gitter (10) Prallbleche aufweist, die in der Draufsicht gekrümmte Linien zeigen, um so ein Muster von sich berührenden Umfangslinien zu bilden.

37. Anlage nach einem der Ansprüche 33 bis 36, dadurch gekennzeichnet, daß das Gitter (10) zwischen benachbarten Prallblechen angeordnete Sperrelemente (49) aufweist, um den Abwärtsstrom von Pulvern aus dem Vorratsbehälter (11) zu versperren.

38. Anlage nach einem der Ansprüche 33 bis 37, dadurch gekennzeichnet, daß die Tiefe der Prallbleche des Gitters derart ist, daß ein Volumen von Pulvern von dem unteren Abschnitt des Vorratsbehälters (11) abgegeben werden kann, das größer ist als das Volumen der zu formenden Fliese.

39. Anlage nach Anspruch 38, dadurch gekennzeichnet, daß das Volumen der abzugebenden Pulver doppelt so groß ist wie das Volumen der zu formenden Fliese.

40. Anlage nach Anspruch 24, dadurch gekennzeichnet, daß die Hülse (36) des Mehrfachverteilers (29) sich abwärts erstreckt, um einen Spender (28) mit einem Maul (28a) parallel zu der Zufuhrseite (3) des Stempelwerkzeuges zu bilden.

41. Anlage nach Anspruch 40, dadurch gekennzeichnet, daß der Abstand zwischen dem Maul und der Zufuhrseite, der die Tiefe (S) der Pulver in den Vorratsbehälter (11) bestimmt, zwischen ungefähr 10 cm und ungefähr 25 cm liegt.

42. Anlage nach Anspruch 33, dadurch gekennzeichnet, daß die Hülse (36) des Mehrfachverteilers (29) einen ringförmigen Ansatz zur Kopplung an einen Träger (37) aufweist, der an einem Förderwagen (38) befördert wird, der doppelseitig auf einem Paar von querverlaufenden Führungsschienen (40) gleitet.

43. Anlage nach Anspruch 32, dadurch gekennzeichnet, daß die Rohrleitungen (30, 31, 32) in ihren oberen Abschnitten flexibel sind, um es zu ermöglichen, daß sie in zugeordnete Pulverbehälter (34, 35, 36) eingeführt werden, die mittels einer Pegelausgleichvorrichtung gespeist werden.

44. Anlage nach Anspruch 32, dadurch gekennzeichnet, daß ein Schlitten (5), auf dem ein Gitter (10) für die Abnahme und den Transfer der Pulver montiert ist, mittels einer Kurbel und einer Kulisse (9) so angetrieben wird, daß er unterhalb des unteren Abschnittes des Vorratsbehälters (11) hin- und herläuft.

45. Anlage nach Anspruch 40, dadurch gekennzeichnet, daß die Hülse (36) an dem Spender (28) längs einer querverlaufenden Ebene (X) schwenkbar montiert ist, die orthogonal zu der Längsachse der Hülse verläuft, um es zu ermöglichen, daß sich diese beim Vorbeilaufen an dem Vorratsbehälter (11) mittels eines Betätigungsgliedes um einen bestimmten Winkel dreht.

46. Anlage nach Anspruch 42, dadurch gekennzeichnet, daß die Rohrleitungen (30, 31, 32, 50, 51, 52, 53, 54, 55) innerhalb der Hülse (36) fixiert sind, wobei der Spender (28) eine Einheit mit dem Förderwagen (38) bildet.

47. Anlage nach Anspruch 19, dadurch gekennzeichnet, daß die Dicke der Prallbleche von Abschnitt zu Abschnitt ein und desselben Prallbleches zwischen wenigen Millimetern und einigen oder mehreren Zentimetern variieren kann.

48. Anlage nach Anspruch 47, dadurch gekennzeichnet, daß die Prallbleche zueinander in der Dicke variieren.

49. Anlage nach Anspruch 40, dadurch gekennzeichnet, daß der Weg der Querbewegung (L) des Spenders (28) gleich der Querabmessung (L1) des Vorratsbehälters (11) minus der Querabmessung (L2) des Spenders selbst ist.

50. Anlage nach Anspruch 19, dadurch gekennzeichnet, daß eine zylindrische, sich drehende Bürste (15) an dem vorderen Teil des Schlittens (5) mittels eines Paares von angelenkten Parallelogrammen montiert ist, die mittels eines Kreuzteiles (17) miteinander verbunden und über einen pneumatischen Zylinder (16) angetrieben sind.

51. Anlage nach einem der vorhergehenden Ansprüche, dadurch gekennzeichnet, daß die Säulen in einer symmetrischen Konfiguration mit einem geraden Querschnitt mit wenigstens einer vorteilhafterweise horizontalen Symmetrieachse (Z3) angeordnet sind, wobei die Konfiguration aufweist:
- wenigstens eine zentrale Säule (30, 30a, 55) zum Führen von Pulvern, die dazu bestimmt sind, die Matrix der Fliese zu bilden, und
- wenigstens ein erstes (31, 51) und ein zweites (32, 52) Paar von sich abwechselnden, gegenüberliegenden Säulen zum Führen der Pulver, die dazu bestimmt sind, die Maserung oder Fleckenverteilung der Fliese zu bilden.

52. Anlage nach Anspruch 51, dadurch gekennzeichnet, daß die symmetrische Konfiguration der Säulen wenigstens eine zentrale Säule (30a, 54, 55) und wenigstens ein sich abwechselndes, gegenüberstehendes Paar von äußeren Säulen (31, 32, 51, 52, 53) umfaßt.

53. Anlage nach Anspruch 51 oder 52, dadurch gekennzeichnet, daß die Symmetrieachse (Z3) des geraden Querschnittes mit der Richtung (Z4) der Querbewegung der Säulen einen Winkel (B2) von zwischen 0° und 180° bildet.

54. Fliese, die durch das in den Ansprüchen 1 bis 18 beanspruchte Verfahren herstellbar ist, mit einer mit Aderung, Maserung und/oder Flächenverteilung versehenen Oberfläche und aus einem trocken geformten keramischen Körper, dadurch gekennzeichnet, daß die Aderung, Maserung und/oder Flächenverteilung sich miteinander vermengen und in die Fliesenmatrix wenigstens bis zu einer merklichen Tiefe der gesamten Dicke eindringen.

55. Fliese nach Anspruch 54, dadurch gekennzeichnet, daß die merkliche Tiefe wenigstens gleich 2 mm ist.

## Revendications

1. Procédé de fabrication de carreaux de céramique moulés à sec, consistant à préparer les poudres, à verser les poudres dans une trémie, à transférer les poudres à un dispositif de pressage, à presser les poudres et à les sécher au four, caractérisé en ce que
- au moins deux types de poudres ou de granules sont chargés dans la trémie et constituent une masse de matériau en granules ou en poudre composée de courants adjacents (33b) qui, au moins dans la partie supérieure de ladite masse, sont distincts les uns des autres ;
- une couche de granules ou de poudre est extraite par gravité du fond de ladite masse de matériau au moyen d'une grille (10) qui forme des ouvertures d'alimentation séparées et sélectionnées (45a), ces ouvertures d'alimentation (45a) étant distribuées en fonction d'un motif de dessin du carreau moulé.

2. Procédé selon la revendication 1, caractérisé en ce que lesdits courants (33b) descendent essentiellement selon un axe vertical.

3. Procédé selon la revendication 1 ou 2, caractérisé en ce que lesdits courants (33b) sont constitués de couches superposées des au moins deux types desdites poudres.

4. Procédé selon la revendication 1, 2 ou 3, caractérisé en ce que ladite masse a la forme d'un prisme ou d'une pyramide tronquée, dont l'axe peut être incliné par rapport au plan vertical, lesdits courants s'entremêlant dans ladite masse.

5. Procédé selon la revendication 4, caractérisé en ce que la profondeur (S) de ladite masse est déterminée par le degré de convergence qui est envisagé entre lesdits courants (33b).

6. Procédé selon la revendication 1 ou 4, caractérisé en ce que lesdits courants (33b) ont essentiellement une section transversale rectangulaire.

7. Procédé selon la revendication 1 ou 4, caractérisé en ce que lesdites ouvertures d'alimentation (45a) sont distribuées selon un motif qui correspond essentiellement à la distribution des veines, des marbrures et des taches présentes dans le carreau moulé.

8. Procédé selon la revendication 1 ou 4, caractérisé en ce que lesdites poudres diffèrent les unes des autres par la couleur, et possiblement par les dimensions du grain.

9. Procédé selon la revendication 1 ou 4, caractérisé en ce que lesdites poudres diffèrent les unes des autres par les dimensions du grain.

10. Procédé selon une ou plusieurs des revendications précédentes, caractérisé en ce que ladite couche inférieure des poudres est au moins égale en volume à celle du carreau non moulé.

11. Procédé selon une ou plusieurs des revendications précédentes, caractérisé en ce que lesdites ouvertures d'alimentation (45a) sont définies par une combinaison quelconque de contours droits.

12. Procédé selon une ou plusieurs des revendication 1 à 10, caractérisé en ce que lesdites ouvertures d'alimentation (45a) sont définies par une combinaison quelconque de contours en courbe reliés ou non par des parties droites.

13. Procédé selon une ou plusieurs des revendications précédentes, caractérisé en ce que lesdites ouvertures d'alimentation (45a) sont obstruées de façon à réduire plus ou moins leur sortie, ce qui facilite l'étalement de la poudre dans le dispositif de pressage.

14. Procédé selon la revendication 3, caractérisé en ce que lesdits courants (33b) stratifiés en couches (6) sont constitués par le dépôt alterné de poudres provenant de colonnes dont les axes sont essentiellement verticaux.

15. Procédé selon la revendication 14, caractérisé en ce que ledit dépôt alterné des poudres est obtenu par un déplacement alterné et possiblement synchrone desdites colonnes dans une direction perpendiculaire à la direction (Y) d'extraction de la couche inférieure des poudres.

16. Procédé selon la revendication 4, caractérisé en ce que ledit dépôt alterné des poudres est obtenu par un déplacement alterné et possiblement synchrone desdites colonnes dans une direction parallèle à la direction (Y) d'extraction de la couche inférieure des poudres.

17. Procédé selon la revendication 15 ou 16, caractérisé en ce que ledit déplacement alterné est complété par une mise en rotation des colonnes autour d'un axe parallèle aux axes des colonnes elles-mêmes, le degré de ladite rotation étant prédéterminé et pouvant atteindre une valeur maximale d'au moins un tour complet.

18. Procédé selon une ou plusieurs des revendications précédentes, caractérisé en ce qu'au moins une desdites colonnes est alimentée de façon intermittente.

19. Usine pour effectuer le moulage de carreaux céramiques par le procédé selon les revendications 1 à 18, comprenant une matrice (12, 13) alimentée au moyen d'une glissière (5) ou d'un chariot, contre-coudé vers et depuis la plaque d'alimentation (3) de la matrice (12) de façon à amener à la matrice elle-même une quantité prédéterminée de poudres extraite par gravité de la sortie inférieure d'une trémie (11) au moyen d'une grille fixée à ladite glissière, caractérisée en ce qu'un distributeur multiple de poudres (29;129), possédant au moins deux canalisations pour alimenter la trémie en colonnes de poudres ou de granules, est monté au-dessus de l'orifice de chargement supérieur de ladite trémie (11) et est entraîné de façon à se déplacer selon un mouvement de va-et-vient, et en ce que la grille (10) est constituée d'une pluralité de chicanes verticales (45, 46, 47, 48) qui forment des ouvertures d'alimentation des poudres séparées et sélectionnées (45a) et qui se conforment à un motif préfigurant celui formé par la distribution des veines, des marbrures et des taches qui sont présentes dans le carreau.

20. Usine selon la revendication 19, caractérisée en ce que ledit distributeur multiple est composé d'un manchon (36) dans lequel au moins deux conduits qui définissent lesdites au moins deux canalisations d'alimentation de la trémie (11) en colonnes de poudre convergent.

21. Usine selon la revendication 20, caractérisée en ce que la section transversale droite dudit distributeur multiple (29) est symétrique par rapport à un axe horizontal (Z3) formant un angle (B2) avec la direction de déplacement du distributeur, ledit angle pouvant varier entre 0 et 180 degrés.

22. Usine selon la revendication 20 ou 21 caractérisée en ce que ledit distributeur multiple (29) dispose de cinq conduits à l'intérieur dudit manchon (36), qui comprennent un conduit central (30a) et deux paires alternées opposées de conduits périphériques (31).

23. Usine selon la revendication 20 ou 21, caractérisée en ce que ledit distributeur multiple (29) dispose de huit conduits à l'intérieur dudit manchon, qui comprennent trois paires alternées opposées de conduits périphériques (51, 52, 53) et deux conduits centraux (54, 55).

24. Usine selon la revendication 19, caractérisée en ce que le distributeur multiple (129) comprend un boîtier (129a) qui couvre essentiellement toute la largeur de la trémie (11), ledit boîtier enfermant une pluralité de conduits (130, 131, 132) dans sa longueur.

25. Usine selon la revendication 24, caractérisée en ce que le distributeur (129) dispose d'une sortie de fond qui fonctionne avec un élément de contrôle du débit.

26. Usine selon la revendication 25, caractérisée en ce que l'élément de contrôle du débit comprend une tablette (151) qui est adjacente à la partie supérieure de la trémie (11) et qui ferme la sortie de fond dudit distributeur.

27. Usine selon la revendication 24, caractérisée en ce que les conduits possèdent des sorties étirables (130a, 131a).

28. Usine selon l'une quelconque des revendications 24 à 27, caractérisée en ce que ladite trémie (11) est pourvue d'une pluralité de pales parallèles (152).

29. Usine selon la revendication 28, caractérisée en ce que les pales peuvent pivoter.

30. Usine selon l'une quelconque des revendications 19 à 29, caractérisée en ce que le distributeur (29;129) est entraîné pour se déplacer selon un mouvement de va-et-vient horizontal.

31. Usine selon la revendication 30, caractérisée en ce que la direction dans laquelle le distributeur est entraîné est parallèle à la direction (Y) de déplacement de la grille.

32. Usine selon la revendication 30, caractérisée en ce que la direction dans laquelle le distributeur est entraîné est perpendiculaire à la direction (Y) de déplacement de la grille.

33. Usine selon une ou plusieurs des revendications 19 à 32, caractérisée en ce que ladite grille (10) dispose de chicanes (45) qui présentent en vue de dessus une combinaison quelconque de lignes courbes ondulées; l'axe (Z1) de chaque chicane formant un angle (B1) par rapport à la direction (Z2, Y) du déplacement de la grille qui est compris entre 0 et 180 degrés, ledit angle n'étant pas nécessairement constant entre les chicanes.

34. Usine selon la revendication 33, caractérisée en ce que ledit angle peut varier d'une section à l'autre pour la même chicane.

35. Usine selon la revendication 33, caractérisée en ce que ladite grille (10) possède des chicanes (47, 48) présentant en vue de dessus une combinaison quelconque de lignes droites.

36. Usine selon la revendication 33, caractérisée en ce que ladite grille (10) comprend des chicanes présentant en vue de dessus des lignes courbes de façon a définir un motif de circonférences adjacentes.

37. Usine selon l'une quelconque des revendications 33 à 36, caractérisée en ce que ladite grille (10) possède des éléments obturants (49) interposés entre les chicanes adjacentes pour obturer la descente des poudres depuis la trémie (11).

38. Usine selon l'une quelconque des revendications 33 à 37, caractérisée en ce que la profondeur des chicanes de ladite grille est telle qu'elle permet d'extraire un volume des poudres de la partie inférieure de la trémie (11) qui est supérieur au volume du carreau à mouler.

39. Usine selon la revendication 38, caractérisée en ce que le volume des poudres à extraire est deux fois plus important que le volume du carreau à mouler.

40. Usine selon la revendication 24, caractérisée en ce que le manchon (36) dudit distributeur multiple (29) se prolonge vers le bas pour constituer un distributeur (28) dont l'ouverture (28a) est parallèle à la plaque d'alimentation (3) de la matrice.

41. Usine selon la revendication 40, caractérisée en ce que la distance entre ladite ouverture et ladite plaque d'alimentation, qui détermine la profondeur (S) des poudres dans la trémie (11), est comprise entre environ 10 cm et environ 25 cm.

42. Usine selon la revendication 33, caractérisée en ce que le manchon (36) dudit distributeur multiple (29) possède une saillie en forme d'anneau pour le relier à une patte (37) montée sur un chariot (38) qui glisse de façon bilatérale sur une paire de rails de guidage transversaux (40).

43. Usine selon la revendication 32, caractérisée en ce que lesdites canalisations (30, 31, 32) ont une partie supérieure souple pour pouvoir les insérer dans des conteneurs de poudre relatifs (33, 34, 35) alimentés au moyen d'un dispositif compensateur de niveau.

44. Usine selon la revendication 32, caractérisée en ce qu'une glissière (5), sur laquelle est montée la grille (10) d'extraction et de transfert des poudres, est entraînée au moyen d'une bielle-manivelle (9) vers et depuis le dessous de la partie inférieure de ladite trémie (11).

45. Usine selon la revendication 40, caractérisée en ce que ledit manchon (36) est monté sur le distributeur (28) en pivotant dans un plan transversal (X) orthogonal à l'axe longitudinal dudit manchon pour lui permettre de tourner transversalement d'un angle prédéterminé par rapport à la trémie (11) au moyen d'un actionneur.

46. Usine selon la revendication 42, caractérisée en ce que lesdits conduits (30, 31, 32, 50, 51, 52, 53, 54, 55) sont fixés à l'intérieur dudit manchon (36), ledit dispensateur (28) étant solidaire dudit chariot (38).

47. Usine selon la revendication 19, caractérisée en ce que l'épaisseur desdites chicanes peut varier d'une section à l'autre pour la même chicane de quelques millimètres à plusieurs centimètres ou plus.

48. Usine selon la revendication 47, caractérisée en ce que l'épaisseur desdites chicanes varie d'une chicane à une autre.

49. Usine selon la revendication 40, caractérisée en ce que la dimension transversale (L) dudit distributeur (28) est égale à la dimension transversale (L1) de la trémie (11) diminuée de la dimension transversale (L2) du distributeur lui-même.

50. Usine selon la revendication 19, caractérisée en ce qu'une brosse cylindrique rotative (15) est montée à l'avant de ladite glissière (5) au moyen d'une paire de parallélogrammes articulés reliés par un élément de traverse (17) et entraînés par un cylindre à commande pneumatique (16).

51. Usine selon l'une quelconque des revendications précédentes, caractérisée en ce que lesdites colonnes sont disposées selon une configuration symétrique dont la section transversale droite comprend au moins un axe de symétrie (Z3) qui est avantageusement horizontal, ladite configuration comprenant :
- au moins une colonne centrale (30, 30a, 55) pour conduire les poudres qui sont destinées à former la matrice du carreau;
- au moins une première (31, 51) et une seconde (32, 52) paires de colonnes alternées opposées destinées à conduire les poudres qui sont destinées à constituer les veines ou les taches du carreau.

52. Usine selon la revendication 51, caractérisée en ce que ladite configuration symétrique des colonnes comprend au moins une colonne centrale (30a, 54, 55) et au moins une paire alternée opposée de colonnes périphériques (31, 32, 51, 52, 53).

53. Usine selon la revendication 51 ou 52, caractérisée en ce que l'axe de symétrie (Z3) de ladite section transversale droite forme un angle (B2) compris entre 0° et 180° avec la direction (Z4) de l'axe transversal des colonnes.

54. Carreau pouvant être obtenu par le procédé selon les revendications 1 à 18, ayant une surface présentant des veines, marbrures, et/ou taches et consistant en un corps céramique moulé à sec, caractérisé en ce que les veines, marbrures et/ou taches s'entremêlent et pénètrent dans la matrice du carreau sur au moins une profondeur essentielle de l'épaisseur totale.

55. Carreau selon la revendication 54, caractérisé en ce que ladite profondeur essentielle est égale à au moins 2 mm.
